

# UNITED STATES PATENT OFFICE.

SAMUEL FIELD, OF LONDON, ENGLAND, ASSIGNOR TO THE METALS EXTRACTION CORPORATION LIMITED, OF LONDON, ENGLAND, A CORPORATION OF GUERNSEY.

## PURIFICATION OF ZINC SOLUTIONS.

1,382,494.

Specification of Letters Patent. Patented June 21, 1921.

No Drawing.

Application filed December 17, 1920. Serial No. 431,482.

To all whom it may concern:

Be it known that I, SAMUEL FIELD, a subject of the King of England, residing at London, England, have invented certain 5 new and useful Improvements in the Purification of Zinc Solutions, of which the following is a specification.

This invention relates to the purification of zinc solutions by the removal therefrom 10 of foreign metals, and has for its object to provide an improved process for this purpose.

According to this invention, the improved process for the purification of zinc solutions, 15 for example, a zinc sulfate solution, from foreign metals comprising treating the solution with a sub-divided metal or alloy more electro-positive than the metallic impurities to be removed (for example, zinc or aluminium or a zinc-aluminium alloy) in the 20 presence of a salt of mercury.

The metal may be employed in granulated form or as powder, or other state of subdivision which is adapted to provide an 25 extended contact surface. For example, zinc fume or blue powder may advantageously be used.

Preferably the zinc solution is acidified, and preferably also the process is carried 30 out with application of heat.

The mercury salt may be added in any convenient way. It may be added as a solution, or the required quantity of the salt 35 itself may be directly dissolved in the zinc solution to be treated, or at a suitable prior stage in the preparation of the latter.

The salts of mercury utilizable include mercuric chlorid and mercuric nitrate, but it 40 will be appreciated that if the zinc is subsequently to be deposited electrolytically the acid radical in the mercury salt must be of such a nature as not to attack the anodes and cause undue disintegration. A suitable salt in this case is mercuric sulfate.

45 It is clear also that when the purified zinc solution is to be electrolyzed, the metal or alloy used in conjunction with the mercury salt must be one whose presence in solution will not be detrimental to the electrolytic 50 process. For this purpose, therefore, zinc in a finely divided form is particularly suitable. When aluminium or an aluminium alloy is used, a certain quantity of this metal 55 passes into solution, but this is in no way detrimental to the subsequent electro-deposi-

tion of the zinc. If desired, however, the aluminium may be subsequently removed concurrently with any iron impurity.

Crude zinc sulfate solutions such as the 60 solutions obtained by the treatment of a zinc ore, previously calcined, if necessary, with sulfuric acid or acid liquor from electrolytic cells, usually contains various foreign 65 constituents, some of which, although present in very small amount, are nevertheless inadmissible if the solution is to be satisfactorily employed for electro-deposition. These foreign constituents include salts of 70 iron, arsenic, antimony, bismuth, copper, cadmium, nickel, cobalt and other less common 75 metals which not infrequently occur in zinc bearing ores.

The present invention may be conveniently exemplified in its application in one 80 way to the purification of a zinc solution of this kind for the subsequent electrolytic deposition of the zinc, it being understood that this example is given for purpose of illustration and not by way of limitation.

To 10 tons of such a solution which has 85 been brought to an acidity of 0.1 to 0.2 per cent., (for instance, by incomplete neutralization, or by complete neutralization for any special purpose, such as the removal of silica, and subsequent acidification with acid or acid liquors), 2 lbs. of mercury in the form of sulfate are added, and then about 40 lbs. of zinc powder, and the liquors are 90 gently stirred while being maintained at a temperature of 70°-100° C.

As a first result of this treatment, mercury 95 is deposited upon the zinc powder which so constitutes a vigorous electro-chemical couple. The metallic impurities, for example, copper, arsenic, antimony, bismuth, cadmium, nickel, cobalt and the rarer metals are precipitated upon the mercury in the 100 form of a sludge which may be readily separated from the liquors by decantation or filtration. This sludge may be subsequently treated in any suitable way for recovery of the mercury, for example, by volatilization of the latter. A considerable proportion of the zinc powder passes into solution and is 105 therefore ultimately recovered by electro-deposition.

If any iron present be not completely precipitated it may be removed by any suitable method either before or after the treatment just described.

Solutions purified by the process herein set forth are particularly suitable for the recovery of zinc by electro-deposition, but as will be readily understood the invention 5 is equally applicable to the preparation of purified zinc solutions for other purposes.

In my prior United States specification, Ser. No. 306,874, I have described a process for the purification of zinc solutions according to which the solutions were treated by immersion therein of amalgamated zinc or aluminium or an amalgamated alloy of these metals. In this process, however, the metal was introduced already amalgamated 10 into the solution, whereas according to the present process amalgamation is actually brought about in the solution undergoing 15 purification.

What I claim as my invention and desire 20 to secure by Letters Patent is:—

1. The herein described process for the purification of a zinc salt solution from foreign metals, which comprises treating the solution with a sub-divided metal more 25 electro-positive than the impurities to be removed, in presence of a salt of mercury.

2. The herein described process for the purification of a zinc salt solution from foreign metals, which comprises treating 30 the solution with a sub-divided alloy more electro-positive than the impurities to be removed, in presence of a salt of mercury.

3. The herein described process for the purification of a zinc salt solution from 35 foreign metals, which comprises treating the acidified solution with a sub-divided metal more electro-positive than the impurities to be removed, in presence of a salt of mercury.

4. The herein described process for the 40 purification of a zinc salt solution from foreign metals, which comprises treating the acidified and heated solution with a sub-divided metal more electro-positive than the impurities to be removed, in presence of a 45 salt of mercury.

5. The herein described process for the purification of a zinc salt solution from foreign metals, which comprises treating 50 the acidified and heated solution with sub-divided zinc in presence of a salt of mercury.

6. The herein described process for the purification of a zinc salt solution from foreign metals, which comprises treating 55 the acidified and heated solution with sub-divided zinc in presence of a salt of mercury in the proportion of about 0.01 per cent. of mercury on the weight of solution treated.

7. The herein described process for the 60 purification of a zinc salt solution from foreign metals, which comprises treating the acidified and heated solution with sub-divided zinc, in presence of mercuric sulfate in the proportion of about 0.01 per cent. of 65 mercury on the weight of solution treated.

8. The herein described process for the purification of a zinc salt solution from foreign metals, which comprises bringing the solution to an acidity of 0.1 to 0.2 per 70 cent., adding mercuric sulfate in the proportion of about 0.01 per cent. of mercury on the weight of solution treated, adding zinc powder and maintaining the solution at a temperature of 70°-100° C. 75

In testimony whereof I affix my signature.

SAMUEL FIELD.